

Nov. 17, 1936.

M. F. PERKINS

2,061,250

COMBINATION DISTILLATION AND LIQUATION FURNACE

Filed Aug. 5, 1932

2 Sheets-Sheet 1



Nov. 17, 1936.

M. F. PERKINS

**2,061,250**

## COMBINATION DISTILLATION AND LIQUATION FURNACE

Filed Aug. 5, 1932

2 Sheets-Sheet 2



## INVENTOR

*Melville F. Perkins*

BY

Attorneys

## ATTORNEYS

## UNITED STATES PATENT OFFICE

2,061,250

## COMBINATION DISTILLATION AND LIQUATION FURNACE

Melville F. Perkins, Woodbridge, N. J., assignor to American Smelting and Refining Company, New York, N. Y., a corporation of New Jersey

Application August 5, 1932, Serial No. 627,589

10 Claims. (Cl. 266—11)

This invention relates to the separation and/or purification of substances by liquation and distillation. The invention particularly relates to apparatus for treating zinc contaminated with 5 lead for the production of zinc vapor in a substantially pure form while simultaneously effecting a concentration of the lead.

The method disclosed herein is claimed in my application Serial No. 736,896, filed July 25, 1934.

10 The invention provides apparatus for continuously and simultaneously subjecting impure spelter to the processes of distillation and liquation in such manner that zinc is continuously distilled from a bath whose low lead content is 15 maintained at a low value by continuous liquation. The invention further provides a furnace having two chambers or compartments connected by appropriate passageways for effecting an intercirculation of molten metal between the compartments, which makes it possible to practise 20 continuous distillation in one compartment while continuously subjecting the metal in the other compartment to liquation.

The invention also consists in certain new and 25 original features of construction and combination of parts hereinafter set forth and claimed.

Although the novel features which are believed 30 to be characteristic of this invention will be particularly pointed out in the claims appended hereto, the invention itself, as to its objects and advantages, and the manner in which it may be carried out, may be better understood by referring 35 to the following description taken in connection with the accompanying drawings forming a part thereof, in which

35 Fig. 1 is a cross section of a furnace embodying the principles of the invention; and

Fig. 2 is a plan view in section of the same 40 furnace on the line 2—2 of Fig. 1.

40 In the following description and in the claims, various details will be identified by specific names for convenience, but they are intended to be as generic in their application as the art will permit.

Like reference characters denote like parts in 45 the several figures of the drawings.

In the drawings accompanying and forming part of this specification, certain specific disclosures of the invention are made for purposes of explanation, but it will be understood that the 50 details may be modified in various respects without departure from the broad aspect of the invention.

Referring now to the drawings, a furnace is shown having walls 10, 11, 12, and 13, roof 14 55 and hearth 15, the latter resting on base mate-

rial 16. Insulation 17 is provided to cover the roof and walls.

• A common wall 18 extending from the roof to the hearth divides the interior of the furnace into two chambers or compartments 19 and 20 which are connected by ports or passageways 21 and 22 extending through wall 18. Fire tubes 23 of suitable refractory material extend through walls 12 and 13 and chamber 20. Passageway 24 connects flue 26 with chamber 19 through port 25. Chamber 19 is provided with a charging port 27 and tap hole 28, while chambers 19 and 20 are provided with exits 29 and 30 respectively. A safety trap 31 is provided in the lower portion of flue 26 by dam 32. Suitable doors not shown are 15 provided for cleaning compartments 19 and 20.

In operation, the invention may be practised as follows. The furnace is charged with the material to be treated and the furnace heated to the proper temperature. For the recovery of 20 zinc from lead, typical substances which may form the charge are raw spelter, galvanizers dross, zinc dross, leady zinc, salvage materials of a similar nature and the like. It is generally preferable to introduce the charge into the liquation compartment through charging port 27, although special cases may warrant direct charging to the distillation chamber. Again, the charge may be introduced either in the liquid or solid state, depending upon circumstances. 25

After melting the charge in the furnace, the respective baths of the liquation and distillation compartments are brought to their appropriate temperatures. The temperature in the liquation compartment is maintained at a value 30 slightly above the melting point of the bath, while in the distillation compartment a sufficient temperature is maintained to insure rapid volatilization of zinc. In general, it has been found that a temperature range of from 430° C. to 500° 35 C. is appropriate for the liquation compartment, while operation of the distillation compartment at temperatures slightly above 900° C. gives excellent results.

Heat may be supplied to the distillation compartment by means of submerged fire tubes constructed of carborundum, graphite, or similar material and which are fired internally with an air-fuel mixture employing the principles of surface combustion. If desired, the fire tubes may 40 be anchored for increased mechanical strength, as by embedding same in the furnace hearth. Other heating means may be employed, but those in which the heat is supplied below the free surface of the bath are preferable. 45

A portion or all of the hot gaseous products of combustion from the fire tubes 23 may be conducted through passageway 24 and into the liquation compartment through port 25 to complete the heat balance in that compartment of the furnace. Combustion gases not used for this purpose are vented through flue 26.

To provide intercirculation and exchange between the liquation and distillation compartments suitable ports 21 and 22 are provided in the dividing wall 18. The rate of circulation may be controlled by the number, size and location of these connecting ports, thus eliminating any necessity for employing a pumping scheme or other method of forced circulation.

By reason of the novel furnace design and the method of operation already described, the bath in the distillation compartment has, at all times, actually and relatively, a low lead content. Hence, in operation, zinc vapor substantially free from lead is volatilized and removed from the compartment through exit 30 from whence it may be condensed to form high grade zinc metal, burned to produce zinc oxide, or otherwise utilized.

Unlike ordinary distillation practices in which the ratio of lead to zinc in the bath must necessarily increase as volatilization of the zinc progresses, the present invention continuously maintains a low ratio of lead to zinc in the bath undergoing distillation. The maintenance of this low lead value is made possible by the intercirculation and exchange effected between the distillation and liquation compartments. As a result of this circulation, the lead left behind in the distillation compartment following the volatilization of the zinc is circulated into the liquation compartment which, as before stated, is substantially cooler than the distillation compartment. At this lower temperature, the lead is less soluble in the zinc and, hence, separates out as a liquid which collects at the bottom of the compartment because of its higher specific gravity.

As the zinc content in the furnace is decreased by volatilization and the lead concentrated in the bottom of the liquation chamber, additional charges of material may be added to the system without interrupting the continuous operation of the furnace. As before stated, the charge may be liquid or solid and may be charged to either compartment, although it will normally be introduced into the liquation compartment. As lead accumulates in the liquation compartment, it may be removed at convenient intervals via top hole 28.

In order to more clearly illustrate the advantages of the present invention and its mode of operation, the following specific example is set forth. Zinc containing from 6% to 10% lead with a trace of iron was charged to the furnace. The liquation compartment was maintained at from 450° C. to 500° C., while the distillation compartment was operated slightly in excess of 900° C., at which temperature volatilization of the zinc proceeded rapidly. Samples of the metal taken from the distillation compartment and the upper stratum of the liquation chamber analyzed 3.06% lead and 3.00% lead, respectively. At the same time, a sample taken from the bottom of the liquation chamber analyzed 96.3% lead, while the volatilized zinc emerging from the distillation compartment analyzed less than .003% lead.

As previously stated, it is possible by the present invention to continuously distill zinc vapor from a bath of low lead content and the above

example illustrates this fact. The importance of constantly maintaining the lead content of the bath in the distillation compartment at a low value, which is made possible by the present invention, is forcibly presented by the following results obtained in making several ordinary distillations from a bottle-shaped retort and employing a small vapor phase filter of crushed rock to prevent splashes of lead in the retort reaching the condensate:

| Analysis of melt in the retort | Analysis of the distilled and condensed zinc |
|--------------------------------|----------------------------------------------|
| Lead % by weight               | Lead % by weight                             |
| 2                              | less than 0.001                              |
| 3                              | 0.003                                        |
| 5                              | 0.01                                         |
| 10                             | 0.012                                        |
| 15                             | 0.02                                         |
| 20                             | 0.03                                         |

This table clearly illustrates the well known fact that as the percentage of lead in a bath from which zinc is being volatilized is increased, the percentage of lead in the vapor and condensate is also increased. By means heretofore described, the present invention, at all times, insures a low lead content in the bath from which the zinc is distilled and thus makes possible the continuous production of substantially pure zinc vapor.

It will be appreciated that while a furnace has been shown having a common dividing wall between the liquation and distillation compartments, various modifications in construction may be effected.

Various heating means and mediums may, of course, be employed for both the liquation and distillation chambers. For example, in one furnace design, burners have been installed in the liquation chamber for melting material charged in the solid state.

Again, while the invention has been described with reference to the separation of lead and zinc, it will be appreciated that the apparatus of the invention may be used to advantage in effecting a large number of separations wherein the appearance of a new phase is produced by change of thermodynamic environment.

While certain novel features of the invention have been disclosed and are pointed out in the annexed claims, it will be understood that various omissions, substitutions and changes may be made by those skilled in the art without departing from the spirit of the invention.

What is claimed is:

1. An apparatus for continuously effecting a separation between zinc and lead by simultaneous distillation and liquation which comprises an insulated furnace having liquation and distillation compartments, a wall common to said compartments, passageways through said wall at least one of same being at the hearth level of the furnace, fire tubes positioned in said distillation compartment and means for conducting waste gas from said fire tubes to said liquation compartment.

2. In the separation of zinc from lead, a furnace having liquation and distillation compartments, means for effecting intercirculation and exchange of molten metal between said compartments, means for heating said distillation compartment and means for conducting waste heat therefrom to said liquation compartment.

3. In apparatus for the separation of lead and zinc, the combination of a liquation chamber, a distillation chamber, sub-surface heating means

- for said distillation chamber and means for intercirculating metal between said liquation and distillation chambers.
4. A furnace for effecting a separation between zinc and lead comprising a liquation chamber, a distillation chamber, a hearth common to both of said chambers, means for maintaining a proper heat balance in said chambers and means for effecting intercirculation and exchange of molten metal between said chambers, said means comprising passageways communicating between said liquation and distillation chambers in different horizontal and vertical planes.
5. A furnace comprising a liquation chamber, a distillation chamber, sub-surface heating means in said distillation chamber and means enabling a thermo-siphonic circulation of material between said compartments.
6. A metallurgical furnace comprising the combination with a roof and hearth, of a wall extending from the roof to the hearth and dividing the interior of the furnace into two compartments, means for circulating metal from each compartment to the other compartment comprising ports in said wall spaced both horizontally and vertically and heating means disposed to deliver heat to the metal in at least one of said compartments below the free surface of the bath.
7. A metallurgical furnace comprising the combination with a roof and hearth, of a wall extending from the roof to the hearth and interiorly dividing the furnace into a pair of compartments, means extending through the said wall for effecting intercirculation and exchange of molten metal between said compartments, fire tubes in one of the compartments for effecting a direct heating thereof and means for conducting hot gases from the fire tubes to the other compartment.
8. A metallurgical furnace comprising the combination with a roof and hearth, of a wall extending from the roof to the hearth and interiorly dividing the furnace into two compartments said wall being provided with passageways enabling intercirculation and exchange of molten metal between said compartments, means for indirectly heating one of the said compartments 10 and a duct leading from said compartment to the other compartment for conducting hot gases from the indirectly heated compartment for heating the other compartment.
9. A metallurgical furnace comprising the combination with a roof and hearth of a wall extending from the roof to the hearth and interiorly dividing the furnace into a pair of compartments, means extending through the said wall for effecting intercirculation and exchange 20 of molten metal between the compartments, means for indirectly heating one of the said compartments, a flue communicating with the indirectly heated compartment and means interconnecting the flue and other compartment for 25 conveying hot gases from the flue to the other compartment for heating the latter.
10. A metal treating furnace comprising two compartments, means for heating metal in one of said compartments by applying heat thereto 30 below its free surface, and means for effecting thermosyphonic circulation of metal between said compartments, said means comprising passageways interconnecting the compartments and spaced both horizontally and vertically. 35

MELVILLE F. PERKINS.